

# United States Patent [19]

Hara et al.

[11] 3,826,886

[45] July 30, 1974

[54] **CONTACT MATERIAL**

[75] Inventors: **Toshito Hara, Kawasaki; Hiroaki Tanaka, Yokohama; Shoichi Shimosato, Kawasaki, all of Japan**

[73] Assignee: **Fujitsu Limited, Kanagawa-ken, Japan**

[22] Filed: **Apr. 5, 1972**

[21] Appl. No.: **241,326**

[30] **Foreign Application Priority Data**

Apr. 15, 1971 Japan ..... 46-23468  
Aug. 30, 1971 Japan ..... 46-66425

[52] U.S. Cl. .... **200/266, 75/138, 75/172 R**

[51] Int. Cl. .... **H01h 1/02, C22c 5/00**

[58] Field of Search ..... **75/172 R, 138; 200/166 C**

[56]

**References Cited**

**UNITED STATES PATENTS**

|           |        |                   |            |
|-----------|--------|-------------------|------------|
| 2,418,710 | 4/1947 | Hensel .....      | 75/172 R   |
| 2,787,688 | 4/1957 | Hall et al. ....  | 75/172 R X |
| 3,428,490 | 2/1969 | Bravo et al. .... | 75/172 R X |

*Primary Examiner*—L. Dewayne Rutledge

*Assistant Examiner*—E. L. Weise

*Attorney, Agent, or Firm*—Nelson E. Kimmelman;  
Maleson Kimmelman

[57]

**ABSTRACT**

A contact material having a high durability is prepared from an alloy consisting of 45 to 85 percent by atom of palladium and 55 to 15 percent by atom of aluminum.

**3 Claims, 7 Drawing Figures**

Fig. 1

## CONSTITUTION OF Pd-AL ALLOY



PATENTED JUL 30 1974

3,826,886

SHEET 2 OF 3

*Fig. 2A*

(Pd)



*Fig. 2B*

(60Pd-40Ag)



*Fig. 2C*

(Pd<sub>2</sub>Al)



*Fig. 2D*

(PdAl)



PATENTED JUL 30 1974

3,826,886

SHEET 3 OF 3



Fig. 3



Fig. 4

1  
CONTACT MATERIAL

The present invention relates to a novel contact material, more particularly, relates to a contact material consisting of a palladium-aluminium alloy and having a high durability.

Electromagnetic relays which include one or more contacts are generally utilized for electrical machinery and apparatus under low level to high level conditions. While electro-magnetic relays having a high durability have heretofore been proposed, such devices have not been found completely satisfactory because of undesirable properties of the conventional contact materials.

Broadly speaking, contact failures may be classified broadly into two classes:

1. increase of contact resistance
2. failure to open. The contact failures as stated above mainly originate from the following sources, high power conditions not considered,
  - a. formation of corrosion products such as oxide or sulfide layers which have low conductivity on the contact surface,
  - b. formation of an organic polymer layer which has low-conductivity on the contact surface,
  - c. material transfer from one of the contact surfaces to the other, and
  - d. erosion of the contact material.

Therefore, in order to provide an excellent contact useful for electrical machinery and apparatus under low level to high level conditions, it is first necessary to provide a contact material having high resistance against corrosion, material transfer and erosion and low activity for formation of organic polymer. Further, it is desirable that the contact material has high hardness and melting point.

Generally, conventional contacts are made of gold, silver, platinum, palladium, rhodium, ruthenium, molybdenum, tungsten and alloys including one or more of the abovementioned metals. However, it is known that although contact material consisting of gold, silver or alloys thereof has a high resistance to corrosion and a low activity for formation of organic polymer, it has undesirably low resistance against material transfer and erosion. It is also known that contact material consisting of a platinum group metal, for example, platinum, palladium, rhodium, ruthenium and alloys thereof, has a high resistance against material transfer and erosion but it has an unfavourable high activity for formation of organic polymer. Further, it is known that a contact material consisting of a metal with a high melting point such as molybdenum, tungsten and alloys thereof has excellent resistance against material transfer and erosion and a low activity for formation of organic polymer while it has an undesirable low resistance against formation of corrosion products.

Generally, intermetallic compounds have a higher hardness and melting point than those of simple metals or nonintermetallic compound alloys because the metal

## 2

atoms in the intermetallic compound are strongly and stably bonded to each other. Accordingly, contact materials consisting essentially of an intermetallic compound have a high resistance to material transfer and erosion. Also, since the intermetallic compounds have poor chemical activity, contact material consisting essentially of them have a poor activity for formation of organic polymer layer and a high resistance to corrosion.

Therefore, the intermetallic compounds have an adoptability for the contact material higher than that of the conventional simple metals or alloys. However, in the case where the intermetallic compound contains no noble metal such as gold, silver and platinum group metals for example, in the case of tungsten carbide (WC) or nickel tin intermetallic compound (NiSn), such intermetallic compounds have an undesirable high tendency to form a stable oxide film on the surface thereof in atmosphere. Accordingly, contacts made up of the intermetallic compounds containing no noble metal frequently suffer from contact failures and thus can not be used under medium or low level conditions.

As is clear from the above description, an ideal contact material which completely satisfies all the above stated requirements has not yet been realized.

An object of the present invention is to provide a contact material satisfying the above-stated requirements that is, having high resistance to corrosion, material transfer, and low erosion and low activity for formation of an organic polymer layer and thus excellent durability.

The object of the present invention can be accomplished by a contact material composed of an alloy consisting of 45 to 85 percent by mol of palladium and 55 to 15 percent by atom of aluminium.

The features and advantages of the present invention will be apparent upon reading the following description and inspecting the accompanying drawings, in which;

FIG. 1 is a phase diagram of palladium-aluminium system,

FIGS. 2A, 2B, 2C and 2D are photographs showing the resistance of Pd metal, Pd-Ag alloy and Pd<sub>2</sub>Al and PdAl compounds to material transfer and erosion,

FIG. 3 is a graph showing the relationship between cumulative failure rate and number of operations for Pd metal and Pd<sub>2</sub>Al and PdAl compounds, and

FIG. 4 shows a circuit for testing the properties of the contact material.

The palladium-aluminium alloys are prepared by an arc-melting method in which a predetermined quantity of palladium (purity: 99.98 percent or higher) is melt-mixed with a balanced quantity of aluminium (purity: 99.999 percent or higher) in an electric furnace using a non-consumption type tungsten anode in an argon atmosphere.

Referring to FIG. 1, the palladium-aluminium alloy includes three intermetallic compounds, Pd<sub>2</sub>Al<sub>3</sub>, PdAl and Pd<sub>2</sub>Al which have properties as shown in Table 1.

Table 1

| Item                     | Material |                    |      |                                 |     |
|--------------------------|----------|--------------------|------|---------------------------------|-----|
|                          | Pd       | Pd <sub>2</sub> Al | PdAl | Pd <sub>2</sub> Al <sub>3</sub> | Al  |
| Melting temperature (°C) | 1558     | 1430               | 1645 | 940                             | 660 |

Table 1

| Item                       | Material       | Pd             | Pd <sub>2</sub> Al | PdAl           | Pd <sub>2</sub> Al <sub>3</sub> | Al |
|----------------------------|----------------|----------------|--------------------|----------------|---------------------------------|----|
| Annealing temperature (°C) | —              | 1200           | 1300               | 800            | —                               |    |
| Hardness before annealing  | —              | 549 Hv         | 560 Hv             | 672 Hv         | —                               |    |
| Hardness after annealing   | 40             | 594 Hv         | 495 Hv             | 668 Hv         | 17 - 23                         |    |
| X-ray micro analysis       | No segregating | No segregating | No segregating     | No segregating | No segregating                  |    |

Note: Hv — Vickers hardness number

As Table 1 clearly shows, the compounds Pd<sub>2</sub>Al and PdAl have an extremely high hardness of about 500 to 600 Hv. The compound Pd<sub>2</sub>Al<sub>3</sub> has a very porous structure which is unsuitable for use as a contact material.

The inventors have discovered that an alloy consisting of 45 to 85 percent by atom of palladium and 55 to 15 percent by atom of aluminium and containing at least one of Pd<sub>2</sub>Al and PdAl, has excellent resistance to corrosion, high hardness and melting point and low chemical activity for formation of organic polymer, and therefore is useful as a contact material having high resistance to material transfer and erosion.

For example, a contact made of the material of the present invention can stably retain a low contact resistance even after the contacts are operated 10<sup>7</sup> times at a contact force of about 4 g at a drive frequency of 1.5 Hz under a contact load of 20 mV - 6 mA in air of a relative humidity of 80 to 90 percent.

If palladium in the alloy is in an amount more than 85 percent by atom, the resultant alloy has a undesirable high activity for the formation of organic polymer on the surface thereof. Also, if the amount of palladium in the alloy is less than 45 percent by atom, the resultant alloy has a low resistance to corrosion, material transfer and erosion.

FIGS. 2A to 2D show the resistance to material transfer and erosion of button-shaped contact made up of a simple Pd metal alloy consisting of 60 parts by atom of Pd and 40 parts by atom of Ag, and intermetallic compounds consisting of Pd<sub>2</sub>Al and PdAl, respectively.

The button-shaped material was made the cathode and the Pd wire was made the anode.

After the button-shaped cathodes were brought into contact with the anodes about 10<sup>5</sup> times under a contact load of 30 V - 3 A at a contact force of 4 g at a drive frequency of 10 Hz in air the appearance of the cathodes and anodes was observed in order to estimate the resistance of the materials to material transfer and erosion.

Referring to FIGS. 2A and 2B, it will be observed that the lower Pd metal and Pd-Ag alloy cathodes were remarkably eroded and transferred to the upper Pd metal mode so as to form a projection on the anode.

In comparison in FIGS. 2C and 2D, the erosion and material transfer of the lower Pd<sub>2</sub>Al and PdAl compound cathodes are distinctly less than those of the Pd metal and Pd-Ag alloy anodes of FIGS. 2A and 2B.

FIG. 3 shows the relationship between the cumulative failure rate of Pd<sub>2</sub>Al and PdAl compounds and the

number of operations saturated xylene vapor in comparison with Pd metal. The term "cumulative failure rate" (C.F.R.) used herein refers to the ratio in percent of the cumulative failure number in excess of the failure level 2  $\omega$  to the cumulative measurement number. The measurement was carried out at a contact force of 4 g, at a drive frequency of 1.5 Hz under a contact load of 20 mV - 6 mA. For every material, 5 to 8 samples were measured.

Referring to FIG. 3, in the measurement of the simple Pd metal contact, the number of contact failures increases after the contact number exceeds 3  $\times$  10<sup>3</sup>, whereas in the measurements of the Pd<sub>2</sub>Al and PdAl compound contacts, no contact failures are observed even after the contact number exceeds 10<sup>6</sup>. From FIG. 3, it is obvious that Pd<sub>2</sub>Al and PdAl compounds have no activity for the formation of organic polymers derived from xylene vapor.

The following examples are intended to illustrate the application of the present invention but are not intended to limit the scope thereof.

#### EXAMPLE 1

An intermetallic compound PdAl was prepared from 50 parts by atom of palladium (purity: higher than 99.98 percent) and 50 parts by atom of aluminium (purity: higher than 99.999 percent) by arc-melting them in a water-cooled copper hearth using a non-consumption type tungsten anode in an argon atmosphere for 30 to 60 seconds. The resultant compound was repeatedly arc-treated in the water-cooled copper hearth on the alternate surfaces thereof in order to homogenize the internal structure thereof. The homogenized compound was annealed at 1300°C for 5 to 6 hours.

The annealed compound was formed into a button-shaped contact strip at 500° to 700°C.

The resultant contact strip had a hardness of 495 Hv.

The two PdAl contact strips were made the anode and cathode, facing each other, of an electromagnetic relay in the circuit as shown in FIG. 4. The contacting operation was carried out in air of a relative humidity of 80 to 90 percent.

Even after 1.5  $\times$  10<sup>5</sup> contactings the PdAl contact showed no contact failure.

In comparison, a simple silver metal contact showed a cumulative failure rate of about 25 percent at 6  $\times$  10<sup>4</sup> contactings.

## EXAMPLE 2

An intermetallic compound  $Pd_2Al$  was prepared from 66.7 parts by atom of pure palladium and 33.7 parts by atom of pure aluminium by the same procedure as Example 1. But the annealing temperature was at  $1200^{\circ}C$ .

The same testing as in Example 1 was applied to the compound  $Pd_2Al$  in air containing 100 p.p.m. of  $H_2S$  gas and having a relative humidity of 80 to 90 percent.

At  $1.3 \times 10^5$  contactings, the  $Pd_2Al$  contact showed a cumulative failure rate of about 54 percent whereas a simple Pd metal contact showed a cumulative failure rate of about 64%.

## EXAMPLE 3

An alloy was prepared from 45 parts by atom of pure palladium and 55 parts by atom of pure aluminium by the same method as is Example 1.

The same tests as in Example 1 were repeated for the above 45 Pd - 55 Al alloy.

Even after  $1.4 \times 10^4$  operations, the 45 Pd - 55 Al alloy contact showed no contact failure. In comparison, a 40 Pd - 60 Al alloy contact showed a cumulative failure rate of 60 percent at  $1.4 \times 10^4$  operations.

## EXAMPLE 4

An alloy was prepared from 60 parts by atom of pure palladium and 40 parts by atom of pure aluminium by the same method as in Example 1.

The resultant 60 Pd - 40 Al alloy was given the same tests as in Example 1 in air of a relative humidity of 80

to 90 percent. Even after  $1.4 \times 10^4$  operations, no contact failures were recorded.

## EXAMPLE 5

5 The same procedure as in Example 1 was repeated using 85 parts by atom of pure palladium and 15 parts by atom of pure aluminium. But the annealing temperature was  $1100^{\circ}C$ .

10 The same testing procedure as in Example 1 was carried out for the above 85 Pd - 15 Al alloy in air containing saturated xylene vapor. Even after  $1.0 \times 10^4$  operations, the 85 Pd - 15 Al alloy contact showed no contact failures.

15 In comparison, a 90 Pd - 10 Al alloy contact showed a cumulative failure rate of 25 percent at  $1.0 \times 10^4$  operations.

What we claim is:

20 1. In an electrical switch having at least one contact, the improvement wherein said contact is composed of an alloy consisting of (1) from 45 percent to 85 percent by atom of palladium and (2) from 55 percent to 15 percent by atom of aluminium.

25 2. An electrical switch as claimed in claim 1, wherein said alloy consists substantially of an intermetallic compound of the formula:  $Pd_2Al$ .

30 3. An electrical switch as claimed in claim 1, wherein said alloy consists substantially of an intermetallic compound of the formula:  $PdAl$ .

\* \* \* \* \*

35

40

45

50

55

60

65

UNITED STATES PATENT OFFICE  
CERTIFICATE OF CORRECTION

Patent No. 3,826,886 Dated July 30, 1974

Inventor(s) Toshito Hara et al

It is certified that error appears in the above-identified patent and that said Letters Patent are hereby corrected as shown below:

Page 1, left column, fourth line from the bottom,  
delete "Aug. 30, 1971 Japan.....46-66425".

Signed and Sealed this  
*thirteenth Day of April 1976*

[SEAL]

Attest:

**RUTH C. MASON**  
*Attesting Officer*

**C. MARSHALL DANN**  
*Commissioner of Patents and Trademarks*